

## THIO FORMAL SYNTHETIC LUBRICANTS

Alfred H. Matuszak, Westfield, and William E. McTurk, Elizabeth, N. J., assignors to Esso Research and Engineering Company, a corporation of Delaware

No Drawing. Application March 16, 1954  
Serial No. 416,688

3 Claims. (Cl. 252—48.6)

This invention relates to synthetic lubricating compositions; particularly the invention relates to synthetic lubricating compositions having outstanding lubricating properties at high and low temperatures and which have the advantage of leaving substantially no combustion chamber deposits in the cylinders of reciprocating engines. More particularly, the invention relates to new and improved synthetic lubricating oils which comprise the formals of organic compounds having at least one free hydroxyl group which is alcoholic in nature and which contains a linkage



wherein  $n$  and  $z$  are small whole numbers, wherein  $x$  and  $w$  are a number from 0 to 8, wherein  $y$  is 1 to 2.

Especially preferred and contemplated in the preferred embodiment of this invention are complex thio formals of the formula



wherein  $A$  and  $B$  may be alike or different and are selected from the group consisting of organic radicals containing from 1 to 60 carbon atoms which correspond to organic compounds containing a hydroxyl group that is alcoholic in nature, wherein  $n$  is a small whole number, wherein  $x$  is a number from 0 to 8, wherein  $y$  is 1 to 2, and wherein  $z$  is a small whole number.  $A$  and  $B$  are preferably selected such that the total number of carbon atoms in the complex thio formal is between about 20 and 130, compounds containing from about 25 to about 100 carbon atoms being especially preferred. The organic hydroxy compounds which serve as a source for the radicals  $A$  and  $B$  will be defined more in detail below.

For use in reciprocating engines, particularly as a lubricant for automotive engines, a lubricating composition must meet several requirements. In order to form an effective lubricating film and to maintain that film at low and high temperatures it must have certain viscosity characteristics. At low temperatures the lubricant must be sufficiently labile to flow through the circulatory system of the equipment and allow movement of lubricated surfaces without an undue power requirement. A lubricant having an ASTM pour point below about 35° F. has sufficient low temperature lability to make it satisfactory in these respects for general use. At high temperatures a lubricant must have sufficient "body" or "thickness" to furnish and maintain a satisfactory lubricating film. It has been found that a lubricant that is satisfactory in this respect will have a viscosity at 210° F. of between about 2 and 60 centistokes, i. e., 32.8 and 280 Saybolt seconds, Universal. To prevent undue lubricant loss, due to volatility and general molecular disintegration and to insure against explosion hazards at higher temperatures

sometimes encountered, a lubricating composition should have a flash point in excess of about 300° F. These requisites are inherent in the term "lubricating compositions," as used in this specification, and the thio formals of this invention are limited to those within these operable ranges. The preferred materials, as contemplated herein and as described in the preferred embodiment hereof, will have an ASTM pour point below about -15° F., a flash point above about 375° F., and will have a viscosity within the range of 2.6 to 13 centistokes, i. e., 35 to 70 Saybolt seconds, Universal, at 210° F.

In general, it has been found that the above listed properties are a function both of molecular structure and of molecular weight. This fact makes it possible, within certain limits, to prepare compositions having similar low and high temperature properties in a variety of ways and also enables the manufacturer to "tailor" a composition to fit a certain set of specifications within rather general limits. This fact also accounts for the large number of organic materials containing alcoholic hydroxyl groups available for preparing the compositions of this invention.

In general the preparation of the thio formals of this invention is accomplished by methods that require conventional techniques and methods. Three general lines of approach may be followed.

(1) All of the reactants may be admixed in the reacting zone and heated to reflux temperature in the presence of an entraining agent such as hexane, heptane or the like. After recovery of the calculated amount of water in this one-step process, the product is washed free of any acidic catalysts and stripped free of unreacted components.

(2) A second approach is to admix  $x$  moles of the thio glycol reactant with  $x-1$  moles of formaldehyde to obtain the central portion of the complex formal, i. e., the portion represented by



In another reacting zone equal mols of an alcohol and formaldehyde are heated to about 60° C. to obtain the hemiformal of the alcohol, i. e.,  $\text{R}-\text{O}-\text{CH}_2-\text{OH}$ . The materials are then blended by adding the thio glycol formal to the alcohol hemiformal and heated to reflux temperature. The product, after removal of the theoretical amount of water, is then washed and stripped as above.

(3) In still a third approach, the hemiformal of the chosen alcohol is first made by heating equal mols of the alcohol and formaldehyde. Then to this is added the desired molar proportion of a thio glycol and formaldehyde and the total mixture heated to reflux temperature to make the hydroxy complex represented by



Two mols of this material is then reacted with one mol of formaldehyde to obtain the product which is purified as above.

The materials used to prepare these formals, that is organic hydroxy compounds containing at least one free hydroxyl group which is alcoholic in character, may be selected from the following partial list. Others, of course, may be used.

I. Unsubstituted alcohols:

A. Monoaliphatic:

1. Aliphatic:
  - a. Methyl alcohol
  - b. Ethyl alcohol
  - c. Propyl alcohol
  - d. Iso propyl alcohol

- e. n-Butyl alcohol
- f. Iso-butyl alcohol
- g. Sec.-butyl alcohol
- h. Tert.-butyl alcohol
- i. n-Amyl alcohol
- j. Iso-amyl alcohol
- k. n-Hexyl alcohol
- l. Iso-hexyl alcohol
- m. 2-ethyl-1-butanol
- n. 2-ethyl-1-hexanol
- o. Octyl alcohol
- p. Iso-octyl alcohol
- q. 2-octyl alcohol
- r. Iso-nonyl alcohol
- s. Decyl alcohol
- t. Lauryl alcohol
- u. Tetradecyl alcohol
- v. Pentadecyl alcohol
- w. Octadecyl alcohol
- x. Allyl alcohol
- y. Crotyl alcohol
- z. Oleyl alcohol
- aa. The terpineols
- bb. C<sub>8</sub> to C<sub>20</sub> Oxo alcohols
- cc. Alcohols derived from the "Synol" process
- dd. Alcohols derived from the oxidation of petroleum fractions
- ee. Alcohols derived from Guerbert's reaction
- ff. Alcohols derived from the hydration of olefins
- gg. Alcohols derived from the "Oxyl" synthesis
- hh. Mixtures of the above
- ii. The corresponding mercaptans

- 2. Aromatic:
- a. Benzyl alcohol
- b. Phenylethyl alcohol
- c. 3-phenyl-1-propanol
- d.  $\alpha$ -Naphthyl carbinol
- e. Cinnamyl alcohol
- f. Diphenyl carbinol
- g. Furfuryl alcohol
- h. Cumic alcohol
- i. Vanillyl alcohol
- j. Piperonyl alcohol
- k. The corresponding mercaptans

## II. Substituted alcohols:

### A. Monohydric:

#### 1. Aliphatic:

- a. Halogenated alcohols—
  - (1) Ethylene chlorohydrin
  - (2) Trifluoro ethanol
  - (3) Propylene chlorohydrin
  - (4) The various chloro-substituted monoethers of polyalkylene glycols
- b. Ethanolamine
- c. 2-amino propanol
- d. 2-nitroethanol
- e. 2-nitropropanol
- f. 2-nitrobutanol
- g. The various glycol monoesters, e. g.—
  - (1) Ethylene glycol monoacetate
  - (2) Propylene glycol monobutyrate
  - (3) Butylene glycol monoaurate
  - (4) Polyethylene glycol monoesters
  - (5) Polypropylene glycol monoesters
  - (6) Polybutylene glycol monoesters
- h. The various glycol monoethers, e. g.—
  - (1) Ethylene glycol mono-methyl ether
  - (2) Propylene glycol mono-butyl ether
  - (3) Butylene glycol mono-lauryl ether
  - (4) Polyethylene glycol mono-ethers
  - (5) Polypropylene glycol mono-ethers
  - (6) Polybutylene mono-ethers
  - (7) Polymethylene glycol mono-ethers
- i. The various glycol mono-formals, e. g. the mixed formals of glycols and alcohols
- j. Hydroxy alkyl cyanides
  - (1) Ethylene cyanohydrin
  - (2)  $\alpha$ -Hydroxy isobutyronitrile
- k. Ethanol morpholine

#### 2. Aromatic:

- a. p-Methoxy benzyl alcohol
- b. The various chlorobenzyl alcohols
- c. The various nitrobenzyl alcohols
- d. 2-aniline ethanol

### B. Other Hydroxy Compounds—

- 1. Esters of hydroxy acids:
  - a. The various lactate esters
  - b. The various glycolate esters
  - c. The various hydroxy stearate esters
- 2. Carbonyl substituted alcohols:
  - a. Hydroxy ketones, e. g.—(1) Hydroxy acetone
  - b. Hydroxy aldehydes, e. g.—
    - (1)  $\alpha$ -Hydroxy adipaldehyde
    - (2)  $\beta$ -Hydroxy propionaldehyde

Particularly desirable organic hydroxy compounds for use in this invention are those highly branched chain aliphatic alcohols prepared by the "Oxo" synthesis. This "Oxo" synthesis may be described as being the catalytic reaction of an olefin with carbon monoxide and hydrogen. The reaction occurs at temperatures in the order of 300°-400° F., at pressures in the range of about 1000 to 3000 p. s. i., in the presence of a suitable catalyst, ordinarily a heavy metal carbonyl such as cobalt carbonyl. The resulting aldehyde is subsequently hydro-

genated to a primary alcohol. This process is described in U. S. Patent No. 2,327,066 issued to Roelen in 1943.

It has been found that particularly desirable alcohols for the formation of the thio formals of this invention can be prepared by the application of the Oxo synthesis to polymers and copolymers of C<sub>3</sub> and C<sub>4</sub> monoolefins. These monoolefins are readily available in petroleum refinery streams and processes for their conversion to liquid copolymers have been worked out by the art. One such process, known as U. O. P. polymerization, consists of passing the olefin-containing stream in liquid phase in contact with an acid catalyst comprising phosphoric acid impregnated on kieselguhr. Other acidic catalysts, such as phosphoric acid or copper phosphate impregnated on silica gel, sulfuric acid, Friedel-Crafts catalysts, activated clays, silica-alumina, copper pyrophosphate, etc., may be used. Suitable conditions when employing phosphoric acid catalysts of the U. O. P. type are temperatures of 300° F. to 500° F., pressures from 250 to 5,000 p. s. i. and feed stocks comprising refinery streams containing propylene and mixed butylenes. Suitable feed stocks, for example, may contain from 15 to 60 mol percent propylenes, from 0.5 to 15 mol percent butylenes, and from 0.1 to 10 mol percent isobutylene, the remaining being saturated hydrocarbons. Other suitable feed stocks are the dimer and trimer of isobutylene.

The preferred Oxo alcohols employed in forming the thio formals of this invention are those having from 8 to 20 carbon atoms derived from olefin copolymers having from 7 to 19 carbon atoms. In preparing these Oxo alcohols the desired olefin fraction is segregated from the crude olefin polymer product by fractionation.

The following table, for example, shows the structure and percent composition of C<sub>8</sub> Oxo alcohols prepared from a C<sub>7</sub> olefin stream which had been fractionated from the products obtained by the phosphoric acid polymerization of refinery gas streams containing propylene and mixed n- and isobutylenes.

| Structure of C <sub>8</sub> Oxo Alcohols Prepared from C <sub>3</sub> -C <sub>4</sub> Copolymer Heptanes | Percent |
|----------------------------------------------------------------------------------------------------------|---------|
|                                                                                                          | 29      |
|                                                                                                          | 25      |
|                                                                                                          | 17      |
|                                                                                                          | 16      |
|                                                                                                          | 2.3     |
|                                                                                                          | 1.4     |
| $\alpha$ -alkyl-alkanols                                                                                 | 4.3     |
| Others                                                                                                   | 5.0     |
|                                                                                                          | 100.0   |

As was stated above, the thio formals of this invention may be considered to have the following general formula



wherein A and B may be alike or different and are selected from the group consisting of organic radicals containing from 1 to 60 carbon atoms which correspond to organic compounds containing a hydroxyl group that is alcoholic in nature, wherein  $n$  is a small whole number, wherein  $x$  is a number from 0 to 8, wherein  $y$  is 1 to 2, and wherein  $z$  is a small whole number. The sum of the carbon atoms in the molecule should be between 20 and 130 and preferably between about 25 and 100.

The group of organic compounds that satisfy the conditions of the above generic formula and that are used to build some of the compounds according to the concept of this invention are monohydric alcohols, thioglycols and organic acids. These compounds may be advantageously combined with formaldehyde to form molecules having the following type formulas, words instead of structures being given to show the components of the complex formals:

Alcohol-(formaldehyde-thiodiglycol) $_z$   
 Thioglycol-(formaldehyde-thiodiglycol) $_z$   
 Polymethylene and polyalkylene glycol-(formaldehyde-thiodiglycol) $_z$   
 Thioglycol monoester-(formaldehyde-thiodiglycol) $_z$   
 Thioglycol monoether-(formaldehyde-thiodiglycol) $_z$

In all formulas given above  $z$  represents a whole number. The acids which may be used to prepare the glycol monoesters may be selected from the following partial list:

|                 |                                                                    |
|-----------------|--------------------------------------------------------------------|
| Acetic          | Methoxy propionic                                                  |
| Propionic       | Ethoxyethoxy acetic                                                |
| Butyric         | Mono-2-ethylhexyl adipate                                          |
| 2-ethyl butyric | Mono-C <sub>8</sub> Oxo sebacic                                    |
| Caproic         | C <sub>8</sub> -C <sub>10</sub> Oxo acids, including bottoms acids |
| 2-ethylhexanoic | Acids derived from petroleum fractions by oxidation                |
| Caprylic        | Acids derived from alcohols and/or aldehydes by caustic fusion     |
| Pelargonic      | Naphthenic acids                                                   |
| Caprie          | Glycolic acid                                                      |
| Lauric          | Lactic acid                                                        |
| Myristic        | Hydroxystearic acid                                                |
| Oleic           |                                                                    |
| Stearic         |                                                                    |

According to a second concept of the instant invention, the molecules set out by the type formulas above that have a free hydroxyl group may be further treated with formaldehyde and joined to another organic compound having a free alcoholic hydroxyl group. This series of compounds, all of which the grouping-(formaldehyde-thiodiglycol) $_x$ ,  $x$  being one or greater than 1, may be shown as follows; the common grouping being designated by Z:

Alcohol-Z-formaldehyde-alcohol  
 Alcohol-Z-formaldehyde-glycol monoester  
 Alcohol-Z-formaldehyde-glycol monoether  
 Glycol monoester-Z-formaldehyde-glycol monoester  
 Glycol monoester-Z-formaldehyde-glycol monoether  
 Glycol monoether-Z-formaldehyde-glycol monoether

By substituting a hydroxy acid monoester such as lactates and glycolates, another series of compounds may be prepared as follows:

5 Hydroxy monoester-Z-formaldehyde-hydroxy monoester  
 Hydroxy monoester-Z-formaldehyde-alcohol  
 Hydroxy monoester-Z-formaldehyde-glycol monoether  
 Hydroxy monoester-Z-formaldehyde-glycol monoester

It will be seen that the above mentioned complex formals all are included under the generic formula:



wherein A and B may be alike or different and are selected

15 from the group consisting of organic radicals containing from 1 to 60 carbon atoms which correspond to organic compounds containing a hydroxyl group that is alcoholic in nature, wherein  $n$  is a small whole number, wherein  $x$  is a number from 0 to 6, wherein  $y$  is 1 to 2, and wherein  $z$  is a small whole number.

20 This concept of the instant invention may be illustrated as follows:

EXAMPLE 1.—COMPLEX THIOFORMAL FROM C<sub>13</sub> OXO ALCOHOL, FORMALDEHYDE AND THIO-DIGLYCOL

Preparation of 1.2 mols of complex thioformal:  
 Alcohol-CH<sub>2</sub>O(thiodiglycol-CH<sub>2</sub>O)<sub>2</sub>-alcohol

25 C<sub>13</sub> Oxo alcohol (480 g.), obtained by oxonation and 30 hydrogenation of tetrapropylene, was heated for 1 hour at 50° C. in the presence of paraformaldehyde (108 g.), heptane (300 g.) and NaHSO<sub>4</sub> (2.2 g.) catalyst. The thiodiglycol (293 g.) was then added and the temperature raised to reflux 95° C. from which it gradually increased to 117° C. after 3 hours. 70 cc. of water was collected. The material was decanted from the catalyst after cooling and washed with three 100 cc. portions of saturated Na<sub>2</sub>CO<sub>3</sub> solution and then three 100 cc. portions of water. The material was then filtered and stripped to a liquid temperature of 186° C. at 0.7 mm. pressure. The liquid thus obtained was clear, had a light straw color and contained 0.93 sulfur (theory=0.94%).

EXAMPLE 2

45 The same complex was prepared as described above but was stripped to 186° C. at only 2.5 mm. pressure. It was light colored and contained 0.91% sulfur.

The complex thioformals prepared as described above 50 possess outstanding lubricating characteristics at both high and low temperatures. Their physical characteristics are set out in Table I below. Included in the table are data on various other complex synthetic lubricants. Blends of these complex lubricants with di-2-ethylhexyl sebacate, all designed to have comparable load carrying 55 ability, are also shown.

TABLE I.—PHYSICAL PROPERTIES OF COMPLEX THIO-FORMAL SYNTHETIC LUBRICANTS

|                        | Complex Thiodiglycol Formal, Ex. I | Complex Thiodiglycol Formal, Ex. II | Complex Thiodiglycol Ester A <sup>1</sup> | Complex Ester B <sup>2</sup> | 75% Complex Ester B, 25% Diester <sup>3</sup> | 10% Complex Thiodiglycol Formal (Ex. I) in 90% Diester <sup>3</sup> | 10% Complex Thiodiglycol Formal (Ex. II) in 90% Diester <sup>3</sup> |
|------------------------|------------------------------------|-------------------------------------|-------------------------------------------|------------------------------|-----------------------------------------------|---------------------------------------------------------------------|----------------------------------------------------------------------|
| Viscosity, Cs. @ ° F.: |                                    |                                     |                                           |                              |                                               |                                                                     |                                                                      |
| 210                    | 7.1                                | 5.5                                 | 7.78                                      | 10.5                         | 8.0                                           | 3.6                                                                 | 3.5                                                                  |
| 100                    | 40.8                               | 25.7                                | 40.9                                      | 52.3                         | 39.9                                          | 14.2                                                                | 13.6                                                                 |
| 0                      | 2,080                              | 760                                 | Crystals                                  | 1,600                        | 1,000                                         | 235                                                                 | 221                                                                  |
| -40                    | 45,000                             | 12,400                              | Solid                                     | 25,150                       | 13,000                                        | 2,000                                                               | 1,820                                                                |
| V. I.                  | 136                                | 156                                 | 148                                       | 152                          | 155                                           | 158                                                                 | 154                                                                  |
| Pour Pt., ° F.         | -60                                | -75                                 | -35                                       | -60                          | -65                                           | -75                                                                 | -75                                                                  |
| Flash Pt., ° F.        | 425                                | 405                                 | 460                                       | 480                          | 435                                           | 425                                                                 | 425                                                                  |

<sup>1</sup> Complex Thiodiglycol Ester A = C<sub>8</sub> Oxo Alcohol—Adipic Acid—Thiodiglycol—Adipic Acid—C<sub>8</sub> Oxo Alcohol.

<sup>2</sup> Complex Ester B = 2-Ethyl hexanol—Sebacic Acid—Polyethylene glycol—Sebacid Acid—2-Ethyl hexanol.

<sup>3</sup> Diester = Di-2 ethyl hexyl sebacate.

TABLE II.—LOAD CARRYING ABILITIES OF COMPLEX SYNTHETIC LUBRICANTS

|                                                                                                             | Test Load, Lbs. |        |
|-------------------------------------------------------------------------------------------------------------|-----------------|--------|
|                                                                                                             | Test 1          | Test 2 |
| Complex Thiodiglycol Formal of Example I                                                                    | 1,500           | 1,600  |
| Complex Thiodiglycol Formal of Example II                                                                   | 1,050           | 1,200  |
| Complex Ester A: C <sub>8</sub> Oxo Alcohol-Adipic Acid-Thiodiglycol-Adipic Acid-C <sub>8</sub> Oxo Alcohol | 1,300           | 1,350  |
| Complex Ester B: 2-Ethylhexanol-Sebacic Acid-Polyethyleneglycol-Sebacic Acid-2-Ethylhexanol                 | 650             | 750    |

## BLENDs OF ABOVE COMPLEXES IN DI-2-ETHYLHEXYL SEBACATE (D. O. S.)

|                                                          |     |     |
|----------------------------------------------------------|-----|-----|
| D. O. S. + 10% Complex Thiodiglycol Formal of Example I  | 700 | 750 |
| D. O. S. + 10% Complex Thiodiglycol Formal of Example II | 700 | 850 |
| D. O. S. + 10% Complex Ester A                           | 750 | 700 |
| D. O. S. + 10% Complex Ester B                           | 600 | 550 |
| D. O. S.                                                 | 450 | 550 |

It will be seen from an examination of the data in Table I that the complex thiodiglycol formals of this invention compare very favorably with the complex esters of the prior art. It will also be noted that the low temperature viscosity of blends of the material of the inventive concept are much superior to the blends containing the known complex esters and possessing comparable load carrying ability. This improvement in the low temperature viscosity property is quite important as will be pointed out in more detail below.

It has been found that the complex thioformals of this invention possess outstanding high load carrying ability superior to that of any of the complex esters hitherto known. The load carrying ability of the materials of this invention are compared with prior art complex esters in Table II. The load carrying test which may be designated as the SAE-SOD test is carried out in the conventional SAE Lubricant Tester employing a 3.4:1 gear ratio. After a run-in period of 2 minutes at a 50 lb. load, the load is increased manually by 50 lbs. every 10 seconds until scuffing occurs. The load at the scuffing point indicates the load carrying ability of the lubricant being tested. Two tests are generally sufficient to characterize the lubricant as shown in Table II.

It will be seen that the load carrying ability of the complex thiodiglycol formals of this invention are outstandingly superior to those of the prior art. This becomes of exceeding importance in preparing blends of diesters for use in aircraft engines. Since the complex thiodiglycol formals of this invention have a much higher load carrying ceiling, lower concentrations can be used to get a high load carrying characteristic in the final blend without seriously increasing the blend viscosities. This is pointed out clearly in the data above. In Table II it is seen that blends of 10% of the complex thioformals of this invention in 90% di-2-ethyl hexyl sebacate have load carrying abilities of from 700 to 850 lbs. From Table I it is seen that these blends have viscosities of less than 2000 centistokes at -40° F. (2000 cs. at -40° F. is considered equivalent to 13,000 cs. at -65° F., the maximum permissible for MIL-L-7808A approval). Both complex esters of the prior art were unsatisfactory at low temperatures and when blends were prepared having a comparable load carrying ability, these too were unsatisfactory because of cloudiness, crystallization or excessive viscosity.

The complex thioformals as described herein may serve as the lubricant base for grease compositions. These synthetic lubricants may be thickened to stable grease structures with conventional grease forming soaps such as lithium soaps of high molecular weight substantially saturated fatty acid, the n-acyl p-amino phenols, silica gels,

treated bentonites and the like. Oxidation inhibitors, rust inhibitors, tackiness agents and other grease addition agents may be added to the complex formal greases. The soap complexes known to the art made by using low molecular weight acid salts may also be used in preparing these grease compositions. If desired the complex formals of this invention may be blended with mineral oil or other synthetic lubricants such as simple bis-formals, complex esters, di-esters such as di-2-ethyl hexyl sebacate, C<sub>8</sub> Oxo adipate, and the like, pentaerythritol tetracaproate, phosphates, siloxanes, silicates, phosphonates and the like and a grease composition which incorporates the desirable characteristics of the blends may be prepared by conventional techniques.

To summarize briefly the instant invention relates to new compositions of matter which have outstanding utility as synthetic lubricating compositions. The materials contemplated may be broadly described as being thioformals of organic materials containing at least one hydroxyl group that is alcoholic in nature. By thioformal is meant materials containing at least a sulfur ether linkage not adjacent to the formaldehyde methylene groups and one or more formal linkages. The structure of the formals of invention may be described as one corresponding to the formula:



wherein A and B may be alike or different and are selected from the group consisting of organic radicals containing from 1 to 60 carbon atoms which correspond to organic compounds containing a hydroxyl group that is alcoholic in nature, wherein n is a small whole number, wherein x is a number from 0 to 8, wherein y is 1 to 2 and wherein z is a small whole number.

The total number of carbon atoms in the molecule should be between about 20 and 130, preferably between about 25 and 100. The compounds that are especially preferred and that are considered to be the preferred embodiment of this invention are those materials which have a kinematic viscosity at 210° F. within the range of from 2 to 60 centistokes, an ASTM pour point of at least as low as 35° F., and a flash point of at least 300° F.

The thioformals of this invention are useful as lubricants, plasticizers, solubilizers, grease bases, insecticides, weed killers, rust preventives, solvents, dewaxing aids, detergents, and as raw materials for many other industrial applications, such as household detergents, fumigants, etc. These new synthetic lubricating oils may be admixed with other lubricating oils, naturally occurring or synthetic, either as concentrates or as finished blends. They are compatible and may be blended with the well known lubricant addition agents such as viscosity index improvers, pour point depressors, detergents, rust inhibitors, antioxidants and the like.

What is claimed is:

1. A synthetic lubricating composition comprising about 90% of di-2-ethyl hexyl sebacate containing combined therein about 10% of a complex thioformal of the formula



2. A synthetic lubricating composition comprising a major proportion of a synthetic carboxylic acid ester having lubricating characteristics and a minor amount sufficient to improve the load carrying ability of said lubricating oil of a complex thioformal having the formula



3. A synthetic lubricating composition according to

claim 2 wherein said carboxylic acid ester is an ester of  
a dicarboxylic acid.

## References Cited in the file of this patent

## UNITED STATES PATENTS

2,472,318 Subkow ----- June 7, 1949

2,503,401  
2,520,748  
2,527,377  
2,570,050  
5 2,577,719  
2,728,748

Mattano ----- Apr. 11, 1950  
Vaughan et al. ----- Aug. 29, 1950  
Patrick ----- Oct. 24, 1950  
Eby ----- Oct. 2, 1951  
Stewart ----- Dec. 4, 1951  
Davis ----- Dec. 27, 1955